

April 18, 1939.

O. EISENHUT ET AL

2,154,893

MANUFACTURE OF ARTIFICIAL THREADS OR THE LIKE

Filed Feb. 15, 1936



Otto Eisenhut  
Hanns Rein  
Hugo Widmann

*Inventors*

By their Attorneys

*Hutz and Joslin*

## UNITED STATES PATENT OFFICE

2,154,893

MANUFACTURE OF ARTIFICIAL THREADS  
OR THE LIKE

Otto Eisenhut, Heidelberg, Hanns Rein, Homberg von der Hohe, and Hugo Widmann, Ludwigshafen-on-the-Rhine, Germany, assignors to I. G. Farbenindustrie Aktiengesellschaft, Frankfort-on-the-Main, Germany

Application February 15, 1936, Serial No. 64,084  
In Germany February 15, 1935

## 3 Claims. (Cl. 18—54)

Our present invention relates to the manufacture of artificial threads or the like.

One of its objects is to provide an improved process of producing artificial threads films or the like from viscose. Further objects will be seen from the detailed specification following hereafter.

It is known that films, threads and the like made from viscose and not subjected to a special 10 aftertreatment have comparatively little strength in wet condition. It has been attempted to increase the wet tenacity of such materials by substituting for the aftertreatment the use of more expensive highly concentrated baths accompanied by stretching, whereby the dry tenacity is increased; however, this process considerably diminishes the extensibility of the material. Moreover, use of highly concentrated baths in itself involves certain technical difficulties and 20 the baths attack cellulose material so that the stability of the material is damaged.

According to this invention we have found that films, threads and the like having a very high tensile strength in the wet state and also good 25 extensibility, may be produced from viscose if the viscose has been ripened so far as to have an ammonium chloride number below 7 to 6 (Hottenroth number). In order to obtain the above effect, the thread must be subjected to tension 30 in a water bath or a bath containing an electrolyte in strong dilution immediately following the coagulation before any or only after traces of cellulose have been regenerated, that is to say while the thread still consists in the main part 35 of xanthogenate. It is essential that the decomposition of the xanthogenate takes place only after the application of tension.

In this manner there is obtained a very homogeneous material which, in the case of thread 40 material, has a substantially cylindrical cross section and does not show even under the highest magnification any or scarcely any difference of structure throughout the whole cross section. If the tension is applied too early, that is to say 45 during the coagulation, then the desired properties are produced to a feeble degree or not at all.

The viscose may be coagulated in the manner 50 described in U. S. Patent No. 2,065,175 by means of water without any addition or with addition of a small quantity of a substance which assists coagulation, while avoiding the use of expensive precipitating baths. Thus a spinning bath having a pH-value of 1.0 to 11 and an osmotic pressure corresponding at most with that of an aqueous solution of 1% of sodium sulfate and 0.2%

of sulfuric acid is suitable. The extension of the coagulated material may be carried out while the material dips into water or in water containing a small quantity of electrolyte. The pH-value of this bath may have the same values as the 5 spinning bath, however, it may be even less than one, so as to correspond with a sulfuric acid content of 1-2%, that is to say, to a pH-value of about 0.8.

With a degree of ripeness corresponding with 10 a Hottenroth number of 2 to 1 the temperature of the water is preferably about 20° C.; if the viscose has been more strongly ripened it is possible to spin even with water of 0° C. If the viscose has been less ripened the spinning bath may 15 have a temperature of 25° C. and more. When spinning threads the bath in which the tension is applied contains preferably traces or a small quantity of electrolyte in order to avoid sticking of the single fibers (for instance, there is used 20 sulfuric acid of 1 to 2 per cent). The tension which is applied to the thread may be produced in various manner, for instance, by bending the thread so that no essential permanent extension of the thread occurs. After having exposed the 25 thread to the tension for producing the high tensile strength in the wet state the xanthogenate is decomposed in the usual manner by means of dilute sulfuric acid with or without the addition of salt whereby lesser concentrations of the 30 decomposing bath than usual may be applied because of the strong self-decomposition of the xanthogenate due to the extremely strong ripening of the viscose.

In the accompanying drawing there is shown 35 an arrangement for spinning in accordance with the invention.

The viscose enters at 1 into a spinning head and is guided to the spinning nozzle 2. The precipitating liquid enters the spinning head through 40 the tube 3 and flows through the spinning funnel 4. In the spinning funnel the viscose is coagulated. When leaving the spinning funnel 4 the thread 8 enters a bath 7 in which rods 9 are provided for imparting tension to the thread 8. 45 After having been tensioned the thread is guided over a rod 10 to a winding up device (not shown). The liquid of the bath 7 is supplied through the tube 5 to a hollow sphere 11 provided with an opening 6.

The process yields surprising products which 50 show extensions of 15-25 per cent. and over in dry and wet condition. The tensile strengths are very good, both in the dry and in the wet state, for example 3 grams per denier dry and 2 55

grams per denier wet, with an extension of 16 per cent. and 18 per cent. respectively. Artificial silk made in accordance with this invention may be aftertreated according to the co-pending application Ser. No. 705,474 now U. S. Patent No. 2,109,306 for Drying.

The following examples illustrate the invention:

*Example 1.*—Viscose having a degree of ripeness corresponding with a Hottenroth number of 1.4 is spun as described in the co-pending application Ser. No. 747,846, filed October 9, 1934 now U. S. Patent No. 2,065,175, through a nozzle having 90 perforations, each 0.8 mm. wide, into a funnel 55 cms. long, the speed of draft being 50 meters per minute and the precipitating bath being water at 22° C.; directly after leaving the funnel the thread and the precipitating water pass into a vessel into which acid has been added, drop by drop, so that the liquid has a pH-value of about 2. For the purpose of producing a tension the thread is guided over rods to the bottom of the vessel and then up again and finally wound on a reel, while being treated with acid. The threads thus obtained and having a titer of 3.5 show the following data:

|                   |                  |          |
|-------------------|------------------|----------|
| Dry tenacity      | grams per denier | 2.5- 2.6 |
| Wet tenacity      | do               | 1.8- 1.9 |
| Extension, dry    | per cent         | 15.3     |
| 30 Extension, wet | do               | 16.2     |

*Example 2.*—When operating as described in Example 1 but bending the thread 4 times for applying tension there is obtained a material which has the same titer as the thread obtained according to Example 1, however it has the following properties:

|                                   |            |      |
|-----------------------------------|------------|------|
| Tensile strength in the dry state | gr./denier | 2.8  |
| Tensile strength in the wet state | do         | 2.3  |
| 40 Extensibility in the dry state | per cent   | 10.5 |
| Extensibility in the wet state    | do         | 10.1 |

What we claim is:

1. A process of producing artificial films, threads and the like of high tensile strength which comprises coagulating viscose having a degree of ripening corresponding with an ammonium chloride number below 7 in an aqueous spinning bath to form xanthogenate containing at most traces of regenerated cellulose, subjecting the coagulated material to tension in a dilute aqueous solution of electrolytes, the osmotic pressure of which corresponds at most with that of an aqueous solution of 1 per cent of sodium sulfate and 0.2 per cent of sulfuric acid, said solution having a pH-value of between 0.8 and 11 while avoiding material permanent extension, and decomposing the material to cellulose hydrate after the application of tension.

2. A process of producing artificial films, threads and the like of high tensile strength which comprises coagulating viscose having a degree of ripening corresponding with an ammonium chloride number below 7 in an aqueous spinning bath having a pH-value of 1.0 to 11 and an osmotic pressure corresponding at most with that of an aqueous solution of 1% of sodium sulfate and 0.2% of sulfuric acid to form xanthogenate containing at most traces of regenerated cellulose, subjecting the coagulated material to tension in an aqueous liquid having a pH-value of 0.8 to 11 and an osmotic pressure corresponding at most with that of an aqueous solution of 1% of sodium sulfate and 2% of sulfuric acid while avoiding material permanent extension, and decomposing the material to cellulose hydrate after the application of tension.

3. A process of producing artificial threads of high tensile strength which comprises spinning viscose having a degree of ripeness corresponding with an ammonium chloride number of 1.4 into a spinning bath of water heated at 22° C. and circulated through a spinning funnel, guiding the spinning bath and the threads into a vessel, mixing said spinning bath with sulfuric acid to have a pH-value of about 2, applying stretch to said threads while in said mixture of sulfuric acid with the spinning bath and winding the threads on a receiving device, while treating them with acid.

OTTO EISENHUT.

HANNS REIN.

HUGO WIDMANN.

45